

## UNITED STATES PATENT OFFICE

ERICH BÖHM, OF VIENNA, AUSTRIA

## TREATMENT OF FELT AND FELT-HAT BODIES

No Drawing. Application filed September 2, 1926, Serial No. 133,298, and in Austria June 1, 1926.

Modern chemistry makes a neat distinction between metal compounds of the first order that is to say compounds in the molecule of which a metal is directly combined with a plurality of atoms of other atoms all of which are of equal nature, and metal compounds of a higher order that is to say compounds the molecules of which result from the combination of a plurality of molecules of compounds of the first order.

An example of a compound of the first order is stannic chloride,  $\text{SnCl}_4$  while an example of a compound of the second order is pink salt



and an example of a compound of the third order is preparing salt or sodium stannate



Such compounds of a higher order are particularly readily formed by metals electro-negative to aluminium and electro-positive to mercury and having a small atom volume and a comparatively high atomic combining capacity such as, iron, zinc, cobalt, nickel, copper, tin, bismuth and before all the metals of the chromium group, namely chromium, tungsten, molybdenum and uranium. Examples of such compounds of higher order, or as they are often called complex compounds are the metal tungstates, as  $[\text{OW}(\text{WO}_4)_3]\text{K}_2$  the metal ammines for instance hexammino-cobalti chloride  $[\text{Co}(\text{NH}_3)_6]\text{Cl}_3$  and its products of substitution, for instance triaquatrimmino-cobalti-chloride



or monochloro-pentammino-cobalti-chloride  $[\text{CoCl}(\text{NH}_3)_5]\text{Cl}_2$  in which the groups combined with potassium or chlorine respectively appear to be self consistent radicles which do not undergo any change if these complex chlorides are converted into nitrates, sulphates, carbonates and the like.

To these compounds of higher order or complex compounds also belong the so called basic chromium salts of very complicated constitution formed in neutralizing chromium compounds split up to a great extent by hy-

drolysis. Thus for instance by neutralizing chromium alum or chromium sulphate it is not chromium hydroxide  $\text{Cr}_2(\text{OH})_6$  that is directly obtained but a series of intermediary compounds namely:

55



down to  $\text{Cr}_4(\text{OH})_{10}\text{SO}_4$  and thereafter chromium hydroxide  $\text{Cr}_2(\text{OH})_6$  is precipitated in the form of a gel.

60

These metal compounds of a higher order or complex metal compounds frequently form colloidal solutions as for instance the chromium compounds just referred to.

I have discovered that the aqueous solutions of metal compounds of a higher order or complex metal compounds as above defined have the property of increasing the lustre of animal hair more particularly of wool hair especially if the solutions are colloidal, and 70 many of these complex metal compounds are known to be tanning agents, that is to say any agents capable of hardening animal collagenous substances. Now my invention consists in treating felt and felt hat bodies with 75 heavy metal compounds of higher order or complex compounds of heavy metals by applying aqueous solutions of such compounds to the felt or felt hat bodies separately or in any stage of their manufacture such as brushing or blocking.

The following is a description of several examples of carrying into practice my invention:

1. I prepare a chromium tanning liquor 85 by neutralizing a normal chromium salt for instance chromium alum such tanning liquor containing about 0.5 to 1% of chromium. This tanning liquor has still to contain about 90 0.1% of sulphuric acid which may be secured either by neutralizing the chromium salt only to the limit indicated or by adding to a liquor more completely neutralized, a sufficient quantity of sulphuric acid or chromium alum. The presence of the small quantity of acid has 95 for its object to prevent the precipitation of chromium hydroxide on the hair which would produce green spots on the felt.

This tanning liquor is heated to about 70 to 80° centigrade and the felt hat bodies are 100

placed into the liquor and left therein under slow agitation for about  $\frac{3}{4}$  to 2 hours according to the quality of the felt. The hat bodies are then taken out and thoroughly rinsed. 5 They have then a beautiful lustre and show a silk like firm hair. They can then be dyed and further treated in the usual manner.

The chromium tanning liquor may also be prepared by the reduction method used by 10 tanners in which a concentrated solution of potassium bichromate and sulphuric acid is reduced by glucose, glycerine, or sulphur dioxide. The green solution contains the chromium compounds of higher order or complex chromium compounds but their percentage varies according to the conditions of reduction and therefore the effect on the felt is somewhat uncertain and besides the felt is liable to be discoloured. Also the commercial 15 chromium tanning liquors or salts may be used.

2. The velour felt hat bodies are placed into a solution of pink salt  $(\text{NH}_4)_2\text{SnCl}_6$ , containing about 1 to 2% of tin and about 0.1 to 0.3% 25 of sulphuric acid and kept there under slow agitation at a temperature of 70 to 80° centigrade for  $\frac{3}{4}$  to 2 hours according to the quality of the hat bodies. The latter are then rinsed and dyed in the usual way.

30 3. The felt hat bodies are placed into a 1% solution of preparing salt,  $\text{Na}_2\text{Sn}(\text{OH})_6$ , and 0.5 to 1% of peroxide of hydrogen at a temperature of 70 to 80° centigrade and kept there under slow agitation for  $\frac{1}{4}$  to 1 hour.

35 Thereby the aspect of the felt becomes smooth and leather like and velour felt hat bodies acquire a high lustre. The addition of peroxide of hydrogen is necessary for preventing the discolouring of the felt, taking place in 40 alkaline solutions. In using this alkaline solution care must be taken to avoid any injury to the felt which might result from a prolonged action of the felt.

4. I prepare an aqueous solution of a tungstate or molybdate soluble in water and containing about 1% of tungsten or molybdenum and add thereto sulphuric acid so that it contains 0.1 to 0.3% thereof. In the case of tungstate solutions the addition of 0.5 to 1% 45 of peroxide of hydrogen is necessary for preventing tungstic acid from being precipitated. The neutral or acid solutions of tungstates or molybdates contain tungsten and molybdenum in the form of complex compounds or 50 compounds of a higher order since the tungstates or molybdates of the first order  $\text{K}_2\text{WO}_4$  and  $(\text{NH}_4)_2\text{MoO}_4$  can exist only in a strongly alkaline solution; the commercial ammonium molybdate for instance has the formula 55  $(\text{NH}_4)_2\text{Mo}_7\text{O}_{24}$  plus  $4\text{H}_2\text{O}$ . The felt hat bodies, more particularly velour felt hat bodies are placed and kept therein for  $\frac{3}{4}$  to 2 hours at a temperature of 70 to 80° centigrade under slow agitation. Thereby velour 60 felt hat bodies having a high lustre are ob-

tained which may be dyed and further treated in the usual manner.

The complex metal compounds as above defined may also be used for brushing velour felt hat bodies or added to such brushing 70 water; they may be also added to the blocking water.

I wish it to be understood that I do not claim the use of potassium bichromate nor the use of ordinary double salts such as potassium aluminium alum. 75

What I claim is:

1. A process for treating felt and felt hat bodies for increasing the lustre thereof consisting in applying thereto an aqueous solution of a complex compound of a heavy metal of the chromium group. 80

2. A process for treating felt and felt hat bodies for increasing the lustre thereof consisting in applying thereto an aqueous solution of a complex compound of chromium. 85

3. A process for treating felt and felt hat bodies for increasing the lustre thereof consisting in applying thereto an aqueous solution of a complex compound of a heavy metal 90 by placing the felt and felt hat bodies into an aqueous solution of such complex salts and keeping them therein at a temperature above room temperature and below the boiling point of water for some time under slow agitation. 95

4. A felt hat body having incorporated into its fibres an inorganic tanning agent.

5. A velour felt hat body having incorporated into its hair an inorganic tanning agent. 100

In testimony whereof I have affixed my signature.

ERICH BÖHM.

105

110

115

120

125

130